# EUROPEAN PATENT SPECIFICATION

(11) **EP 0 458 591 B1**
(45) Date of publication and mention of the grant of the patent: **18.10.1995**
(21) Application number: 91304577.9
(22) Date of filing: 21.05.1991
(51) Int. Cl.: B24D 3/00, B24D 13/14

(54) **Buffing pad**
Schwabbelpolster
Tampon de polissage

(30) Priority: 21.05.1990 GB 9011343
(43) Date of publication of application: 27.11.1991
(73) Proprietor: MINNESOTA MINING AND MANUFACTURING COMPANY, St. Paul, Minnesota 55133-3427 (US)
(72) Inventor: Foster, James, c/o Minnesota Mining and, Atherstone, Warwicks CV9 1PJ (GB)
(74) Representative: Bowman, Paul Alan

(56) References cited:
- EP-A- 0 333 611
- DE-A- 3 903 204
- GB-A- 1 083 547
- US-A- 3 112 584

## Description

The present invention relates to buffing pads and in particular to buffing pads adapted to be releasably engaged with buffing apparatus having an attachment surface of the hook-face type.

EP-A-0333611 discloses a polishing disc for marble or similar substances consisting of a disc of metal mesh or the like, having one face with at least one corrugated metal gauze by which it is hooked to a drive plate of a polisher or similar device, equipped with a "velcro" or similar fastening system, and on its other face at least one corrugated metal gauze with characteristics that may or may not be different from those of the corrugated gauze(s) on the first face.

GB 1,083,547 discloses a polishing head for glass or the like comprising disk mounting means and polishing pad means, one of the means having a plurality of loops thereon removably engaging a plurality of hook elements on sheet material of the other of the means whereby the polishing pad means can be readily removed from the mounting means.

US-A-5,030,496 discloses a flexible and resilient, fibrous, nonwoven, surface treating article comprising an open, lofty, nonwoven fibrous web formed of entangled, synthetic, organic fibres bonded together at points where they contact one another by a cured, tough, fracture resistant, substantially homogenous, primary binder resin comprising plasticized vinyl resin and polymerized amine-formaldehyde derivative.

US-A-3,703,739 discloses surface working pads formed of open non-woven three-dimensional web material, as typified by the so-called nylon floor pads. The pads are releasably retained on a driving disc or brush block in a stack in which adjacent pads are held together by double face, flexible, pad holding material which provides a multitude of projecting tiny adhering filaments.

US-A-5,001,804 discloses circular buffing pads or buffs adapted to be releasably engaged with backup pads. A buff adapted for self centering engagement with a backup pad comprises a circular body with a first fastener portion on its face. The buff includes a stiff flexible backing having a generally planar circular central portion and an annular flange only slightly larger than the diameter of the backup pad projecting from one side surface of its central portion, a second fastener portion fixed on the side surface of its central portion and adapted for engagement with the fastener portion on the backup pad, and a multiplicity of projecting tufts having central portions adhered in the backing by a thermoplastic adhesive that melts and adheres at a temperature under 100°C.

US-A-4,758,290 discloses a buffing pad comprising a fabric pile for application against a workpiece, a backside carrying the fabric pile, loop means carried centrally of the pad and against the backing side, and enveloping the periphery of the loop means. The buffing pads may be any of those of known type having various fabrics such as natural wool strands, lambswool, synthetic fibres, and the like, as well as cloth materials such as terry cloth and the like.

One construction of buffing pad commonly used in the automobile trade comprises a web of non-woven fibers. The attachment surface of the back-up pad of buffing apparatus, such as rotary and orbital buffers, is provided with a multiplicity of projecting, resiliently-flexible filaments bearing at the distal end thereof a bulbous substantially semi-spherical head or hook. This surface is commonly referred to as a hook-face attachment surface. When the buffing pad is placed against the attachment surface the head or hooks of the attachment surface mechanically interlock with the non-woven fibers of the pad to secure the pad in position. As such, this type of buffing pad has found great favor by allowing the user to easily reposition the pad or remove it entirely for replacement.

It has been found that commercially available buffing pads manufactured from thick fibers having a caliper of about 17 dtex while providing good adhesion to the back-up pad and good buffing properties for use on original automotive equipment manufacture painted surfaces tend to be too aggressive when used on other paint surfaces, e.g., the softer after-market air-dried or low-bake paints normally used in body repair shops. Buffing pads formed from finer fibers, e.g., having a dtex of 6.7, while proving acceptable for use with softer paint finishes are found to have a poor adhesion for the hook-face attachment surfaces of the back-up pad and are often displaced during use.

The present invention provides a buffing pad suitable for use with softer paint products but having an improved adhesion for buffing apparatus having a hook-face attachment surface.

According to the present invention there is provided a buffing pad laminate having one side adapted to be releasably engaged with a buffing apparatus having a hook-face attachment surface and an opposite side for buffing, the buffing pad laminate comprising a non-woven buffing layer comprising crimped fibres having a fibre thickness of up to 11 dtex and a fibre length of from 40 to 200mm, a non-woven attachment layer comprising crimped fibres having a fibre thickness greater than 11 dtex and a fibre length of at least 40mm, in which the buffing layer and the attachment layer are secured together by intermingling fibres of the buffing layer with fibres of said attachment layer, the buffing pad having a density of from 0.1 to 0.3 g/cm³, and a thickness of from 3 to 8mm.

The buffing pads of the invention comprise a multilaminate construction formed from the combination of thick and thin fibres, with a preponderance of thick fibres forming an attachment layer to provide good adhesion to the attachment surface of the back-up pad, and a preponderance of thin fibres forming a buffing layer to provide a milder buffing action suitable for use with softer substrates, the fibres of each layer being intermingled to secure the layers together.

The total thickness of the buffing pad varies with its intended use in the range from 3 to 8mm, preferably in the range from 4 to 6mm, with a typical value being about 5mm. Although buffing pads may be constructed outside of this range, pads less than 3mm thick tend to lack sufficient structural integrity for prolonged use and for pads greater than 8mm thick there is no further practical advantage to be gained without the cost of manufacture becoming uneconomical.

The buffing pads comprise a laminate of a buffing layer bonded to an attachment layer. The non-woven, crimped fibres of the attachment layer provide a surface having a multiplicity of loops suitable for engagement with the filament of a hook-face attachment surface. The buffing layer generally comprises at least 50% of the total pad thickness, normally in the range from 50 to 75% with the remainder comprising the attachment layer. Preferably, the buffing layer comprises in the range from 50 to 65% of the total pad thickness and the attachment layer in the range from 50 to 35%.

The buffing pads have a density in the range from 0.1 to 0.3 g/cm³, preferably in the range from 0.12 to 0.18 g/cm³, with a typical value in the range from about 0.15 to 0.16 g/cm³.

The buffing layer is composed of thin fibers having a caliper of up to 11 dtex, preferably up to 8 dtex, with a typical value being about 6.7 dtex. The length of the individual fibers is at least 40 mm to reduce linting during use, i.e., detachment of individual fibers. The length of the buffing layer fibers is in the range from 40 to 200 mm, preferably in the range from 40 to 80 mm, with a typical value of about 60 mm. Fibers of greater than 200 mm length tend to present handling difficulties during manufacture.

The attachment layer comprises thicker fibers having a caliper of greater than 11 dtex, preferably at least 13 dtex, with a typical value of about 17 dtex. The attachment layer may comprise solely "thick" fibers or a blend of both thick and thin fibers may be used. The fibers of the attachment layer generally have a length in the range from 40 to 200 mm, preferably in the range from 60 to 100 mm, with a typical value being about 75 mm.

Suitable crimped fibers are known in the art and are commercially available in a range of standard dtex, such as, for example, 1.5, 3.3, 6.7, 8.9, 11, 13, 17, 23 and 30. The fibers may be formed from natural materials, such as, for example, wool, cotton and other cellulosic materials, and synthetic polymers and co-polymers such as, for example, polyamides, polyacrylates, polyesters, nylons and viscose. Each layer may comprise a single fiber type or a mixture of two or more fibers.

It is preferred to fabricate the buffing layer from fibers of a different color or tonal contrast to those used in the attachment layer as this is found to provide a simple and effective means of indicating to the user, the correct orientation of the buffing pad. This may be conveniently achieved by employing some colored fibers in the attachment layer, e.g., 30% colored fibers and 70% white fibers.

The buffing and attachment layers are secured to each other by intermingling fibres from the two layers e.g., by needle punching the laminate. In order to avoid fibers from the attachment layer extending through the surface of the buffing layer, which would impart an aggressive nature to the buffing surface, the needle punching is preferably effected from the buffing layer causing fibers from the buffing layer to be intermingled with the fibers in the attachment layer. Needle punching is a conventional technique in the manufacture of certain types of non-woven materials. Generally, needle punching of the laminate is effected using needle size numbers in the range from 38 to 32. Typically the needle punching maybe effected to provide approximately 500 apertures/cm².

The individual buffing and attachment layers may be formed from the filaments by a similar needle punching process. Generally, the fibers are carded, air laid as a web, compressed by calender rollers and needle punched to form a self-supporting material. The buffing layer and/or the attachment layer may be formed by combining two or more of such webs of material and needle punching.

The composite comprising the buffing and attachment layers may undergo a further treatment in which a bonding agent is applied throughout the composite to provide further structural integrity and to reduce the propensity of the material to lint during use. The bonding agent is conveniently applied by immersion the material in a bath of liquid bonding agent followed by drying, e.g., in a air tunnel or with infrared heaters. Suitable commercially available bonding agents include, for example, polyvinyl alcohol, polyvinyl acetate, acrylic emulsions, butadiene-acrylo nitrile copolymer and other water-dispersible lattices. The bonding agents are usually employed as a 15 to 25%, typically 20% by weight of solids dispersed in water.

The buffing pads of the invention are suitable for use in any type of buffing apparatus having a hook-face attachment surface. The buffing apparatus may be of the rotary or orbital type or it may be in the form of a block or pad for hand use. The hook-face attachment surface comprises a multiplicity of projecting, resiliently-flexible filaments having at the distal end thereof a head or hook-like projection. Suitable hookface attachment surfaces generally comprise in the range from 50 to 120 filaments/cm², preferably in the range from 60 to 100 filaments/cm², the filaments having an average height in the range from 0.75 to 1.5 mm, preferably in the range from 0.9 to 1.3 mm; an average diameter in the range from 0.15 to 0.35 mm, preferably in the range from 0.2 to 0.3 mm; and an average head diameter in the range from 0.4 to 0.75 mm, preferably in the range from 0.55 to 0.65 mm.

Suitable materials are commercially available under the trademarks "lH2" from Kanebo Bell-Touch Ltd. of Osaka, Japan, "HOOK-IT" from Minnesota Mining and Manufacturing Company of St. Paul, MN and "KLETTOGRIP" from Gottlieb Binder GmbH and Co. of Holzgerlingen, Germany. Typical rotary buffer apparatus will utilize a circular buffing pad having a diameter in the range from 50 to 200 mm.

A typical process for the manufacture of a buffing pad in accordance with the invention comprises:
providing a source of crimped fibers suitable for the buffing layer, e.g., having a caliper of 6.7 dtex and an average fiber length of 60 mm, e.g., in the form of a bale;
carding the fibers and air laying the carded fibers in one or more layers onto a moveable support member to form a fleece of substantially horizontally aligned fibers;
calendering the fleece and optionally needle punching from either one or both sides to form a non-woven web of fibers suitable for the buffing layer;
providing a source of crimped fibers suitable for the attachment layer, e.g., having a caliper of 17 dtex and an average fiber length of 75 mm and repeating the above steps to form a non-woven web of fibers suitable for use as the attachment layer;
overlaying the web to form the attachment layer with at least one web to form the buffing layer and needle punching the combined layers from the buffing layer to the attachment layer to form a laminate of the buffing and attachment layers;
optionally repeating the needle punching step one or more times to increase the structural integrity and density of the resulting material;
passing the resulting laminate through a bath of an aqueous-based latex, e.g., 20% by weight solids-of butadiene-acrylo nitrile copolymer in water, drying the laminate, and cutting to the desired size to form the buffing pad.

The web of fibers to form the attachment layer is preferably needle punched from one side only in order to attain a surface having a multiplicity of exposed loops of fiber which form an effective attachment surface for co-operation with the hook-face surface.

Objects and advantages of this invention are further illustrated by the following example, but the particular materials and amounts thereof recited in this example, as well as other conditions and details, should not be construed to unduly limit this invention.

### Example

A buffing pad having 60 mm long crimped 6.7 dtex viscose fibers (commercially available in crimped form from the VFG Company of Giengen/Brenz, Germany) on the buffing side and 60 mm long crimped 17 dtex viscose fibers (commercially available in crimped form from the VFG Company) on the attachment side was prepared. Using conventional equipment, each of the 6.7 dtex fibers and 17 dtex fibers were carded and air laid in a layer to provide fleeces of substantially horizontally aligned fibers. Each fleece was then calendered to provide a nonwoven web comprising 6.7 dtex fibers and a nonwoven web comprising 17 dtex fibers. The web comprising the 6.7 dtex fibers (buffing web) was overlaid onto the web comprising the 17 dtex fibers (attachment web). The webs were combined by needle punching from the buffing web through the attachment web using a needle having a needle size number of 32 (specifically the needle was 15 x 18 x 8.9 cm RB Gepraeght (= Embossed)). The needle punching provided about 500 apertures/cm. The resulting diameter of the resulting buffing pad was about 12.7 cm (5 inches).

A conventional automobile hood was sprayed with a 2K polyurethane two component paint (commercially available from Herberts of Wuppertal, Germany). The paint was cured by heating the painted hood in an oven at a temperature of about 60°C for about 30 minutes.

To simulate a repair, a portion of the painted hood (about 2 cm by about 2 cm) was hand sanded using a 3.65 cm diameter scallop disc having 9 micrometer abrasive particles thereon (commercially available under the trademarked designation "FINESSE-IT 9 MICRON SCALLOP DISC" from the 3M Company of St. Paul, MN), which was mounted to a sanding hand block (commercially available under the trademarked designation "FINESSE-IT HAND BLOCK" from the 3M Company).

The buffing pad was attached to a conventional rotary air polishing machine with a soft, hook faced backup pad (commercially available under the trademarked designation "FINESSE-IT BACKUP PAD" from the 3M Company). The sanded area of the paint was buffed using the buffing pad and a buffing compound (commercially available under the trademarked designation "FINESSE-IT FINISHING COMPOUND" from the 3M Company). The free spinning rotational speed of the air polishing machine was about 1800 rpm. The buffing time was about 10 seconds.

The gloss of the buffed and unbuffed (i.e., a portion of the painted hood as sprayed and cured) were measured using a gloss meter (commercially available under the trade designation "NOVO-GLOSS NG 60C AUTO GLOSS METER" from Rhopoint Surface Instruments of Oxted Surrey, UK). The gloss of the buffed area measured at an angle of about 60 degrees was about 90 to 92, whereas the gloss of the unbuffed area was about 92.

The buffing pad was detached from the backup pad by pulling the pad perpendicularly from the pad-backup pad interface.

## Claims

1. A buffing pad laminate having one side adapted to be releasably engaged with a buffing apparatus having a hook-face attachment surface and an opposite side for buffing, the buffing pad laminate comprising a non-woven buffing layer comprising crimped fibres having a fibre thickness of up to 11 dtex and a fibre length of from 40 to 200mm, a non-woven attachment layer comprising crimped fibres having a fibre thickness greater than 11 dtex and a fibre length of at least 40mm, in which the buffing layer and the attachment layer are secured together by intermingling fibres of the buffing layer with fibres of said attachment layer, the buffing pad having a density of from 0.1 to 0.3 g/cm³, and a thickness of from 3 to 8mm.

2. A buffing pad as claimed in Claim 1 characterised in that the buffing pad is circular and has a diameter of from 50 to 200mm.

3. A buffing pad as claimed in Claim 1 or Claim 2 characterised in that the buffing layer comprises in the range from 50 to 75% of the total pad thickness and the attachment layer comprises in the range from 50 to 25% of the total pad thickness.

4. A buffing pad as claimed in any preceding Claim characterised in that the buffing layer fibres and the attachment layer fibres are independently selected from wool, cotton cellulose-based fibres, viscose fibres, polyamide fibres, polyacrylate fibres, polyester fibres and nylon fibres.

5. A buffing pad as claimed in any preceding Claim characterised in that the fibres of the buffing layer have a dtex value up to 8 and the fibres of the attachment layer have a dtex value of at least 13.

6. A buffing pad as claimed in any preceding Claim further characterised in that a bonding agent is distributed between the fibres.

7. A buffing pad as claimed in any preceding Claim characterised in that the said intermingling of fibres of the buffing layer with fibres of the attachment layer is a result of needle punching.

8. Buffing apparatus comprising hook-face attachment surface comprising a multiplicity of projecting, resiliently-flexible filaments having at the distal end thereof a head or hook-like projection and a buffing pad as claimed in any preceding Claim.

9. A process for manufacturing a buffing pad, the process characterised by the step of securing a non-woven buffing layer comprising fibres having a fibre thickness of up to 11 dtex and a fibre length of from 40mm to 200mm to a non-woven attachment layer comprising fibres having a fibre thickness greater than 11 dtex and a fibre length of 40mm, by intermingling fibres of the buffing and attachment layers.

10. A process as claimed in Claim 9 characterised in that the intermingling is caused by needle punching.

11. A process as claimed in Claim 9 or Claim 10 characterised in that a bonding agent is applied to the fibres of the buffing layer and the attachment layer.

## Patentansprüche

1. Schwabbelpolsterlaminat, dessen eine Seite mit einer Schwabbelvorrichtung mit einer mit Haken versehenen Befestigungsfläche lösbar in Eingriff gebracht werden kann und dessen entgegengesetzte Seite für eine Schwabbelbearbeitung geeignet ist, wobei das Schwabbelpolsterlaminat aufweist: eine ungewebte Schwabbelbearbeitungsschicht mit gekräuselten Fasern mit einer Faserdicke von bis zu 11 dtex und einer Faserlänge von 40 bis 200 mm und eine ungewebte Befestigungsschicht mit gekräuselten Fasern mit einer Faserdicke von mehr als 11 dtex und einer Faserlänge von mindestens 40 mm, wobei die Schwabbelbearbeitungsschicht und die Befestigungsschicht durch Vermischen von Fasern der Schwabbelbearbeitungsschicht mit Fasern der Befestigungsschicht miteinander verbunden sind und wobei das Schwabbelpolster eine Dichte von 0.1 bis 0.3 g/cm³ und eine Dicke von 3 bis 8 mm aufweist.

2. Schwabbelpolster nach Anspruch 1, dadurch gekennzeichnet, daß das Schwabbelpolster kreisförmig ist und einen Durchmesser von 50 bis 200 mm aufweist.

3. Schwabbelpolster nach Anspruch 1 oder 2, dadurch gekennzeichnet, daß die Dicke der Schwabelbearbeitungsschicht 50 bis 75% der Gesamtdicke des Polsters und die Dicke der Befestigungsschicht 50 bis 25% der Gesamtdicke des Polsters beträgt.

4. Schwabbelpolster nach einem der vorangehenden Ansprüche, dadurch gekennzeichnet, daß die Fasern der Schwabbelbearbeitungsschicht und der Befestigungsschicht unabhängig voneinander aus Wollfasern, Baumwollfasern, auf Zellulose basierenden Fasern, Viskosefasern, Polyamidfasern, Polyacrylsäureesterfasern, Polyesterfasern oder Nylonfasern ausgewählt werden.

5. Schwabbelpolster nach einem der vorangehenden Ansprüche, dadurch gekennzeichnet, daß die Fasern der Schwabbelbearbeitungsschicht einen dtex-Wert bis zu 8 und die Fasern der Befestigungsschicht einen dtex-Wert von mindestens 13 aufweisen.

6. Schwabbelpolster nach einem der vorangehenden Ansprüche, ferner dadurch gekennzeichnet, daß zwischen den Fasern ein Haftvermittler verteilt ist.

7. Schwabbelpolster nach einem der vorangehenden Ansprüche, dadurch gekennzeichnet, daß die Fasern der Schwabbelbearbeitungsschicht und die Fasern der Befestigungsschicht durch Vernadeln miteinander vermischt werden.

8. Schwabbelvorrichtung mit einer mit Haken versehenen Befestigungsfläche mit mehreren hervorstehenden elastisch-flexiblen Fäden, an deren distalem Ende ein Kopf oder ein hakenähnlicher Vorsprung angeordnet ist, und einem Schwabbelpolster nach einem der vorangehenden Ansprüche.

9. Verfahren zum Herstellen eines Schwabbelpolsters mit dem Schritt: Befestigen einer ungewebten Schwabbelbearbeitungsschicht mit Fasern mit einer Faserdicke von bis zu 11 dtex und einer Faserlänge von 40 bis 200 mm an einer ungewebten Befestigungsschicht mit Fasern mit einer Fasserdicke von mehr als 11 dtex und einer Faserlänge von 40 mm durch Vermischen der Fasern der Schwabbelbearbeitungsschicht und der Befestigungsschicht.

10. Verfahren nach Anspruch 9, dadurch gekennzeichnet, daß das Vermischen durch Vernadeln durchgeführt wird.

11. Verfahren nach Anspruch 9 oder 10, dadurch gekennzeichnet, daß auf die Fasern der Schwabbelbearbeitungs- und der Befestigungsschicht ein Haftvermittler aufgebracht wird.

## Revendications

1. Stratifié pour tampon de polissage dont une face est prévue pour venir en prise libérable avec un appareil de polissage présentant une surface d'attache à face d'accrochage, et dont la face opposée est prévue pour le polissage, le stratifié pour tampon de polissage comprenant une couche de polissage non-tissée à fibres frisées ayant une épaisseur de fibre jusqu'à 11 dtex et une longueur de fibre de 40 à 200 mm, et une couche d'attache non-tissée à fibres frisées ayant une épaisseur de fibre supérieure à 11 dtex et une longueur de fibre d'au moins 40 mm, la couche de polissage et la couche d'attache étant fixées l'une à l'autre par enchevêtrement de fibres de la couche de polissage avec des fibres de la couche d'attache, le tampon de polissage ayant une densité de 0,1 à 0,3 g/cm³ et une épaisseur de 3 à 8 mm.

2. Tampon de polissage suivant la revendication 1, caractérisé en ce que le tampon de polissage est circulaire et a un diamètre de 50 à 200 mm.

3. Tampon de polissage suivant la revendication 1 ou la revendication 2, caractérisé en ce que la couche de polissage constitue de 50 à 75% de l'épaisseur totale du tampon et la couche d'attache constitue de 50 à 25% de l'épaisseur totale du tampon.

4. Tampon de polissage suivant une quelconque des revendications précédentes, caractérisé en ce que les fibres de la couche de polissage et les fibres de la couche d'attache sont choisies indépendamment parmi laine, coton, fibres à base de cellulose, fibres de viscose, fibres de polyamide, fibres de polyacrylate, fibres de polyester et fibres de nylon.

5. Tampon de polissage suivant une quelconque des revendications précédentes, caractérisé en ce que les fibres de la couche de polissage ont une valeur de dtex pouvant atteindre 8 et les fibres de la couche d'attache ont une valeur de dtex d'au moins 13.

6. Tampon de polissage suivant une quelconque des revendications précédentes, caractérisé en outre en ce qu'un liant est distribué entre les fibres.

7. Tampon de polissage suivant une quelconque des revendications précédentes, caractérisé en ce que ledit enchevêtrement de fibres de la couche de polissage avec des fibres de la couche d'attache est produit par aiguilletage.

8. Appareil de polissage comprenant une surface d'attache à face d'accrochage, comportant une multiplicité de filaments saillants élastiquement flexibles dont l'extrémité distale porte une tête ou un crochet, et un tampon de polissage suivant une quelconque des revendications précédentes.

9. Procédé de fabrication d'un tampon de polissage, le procédé étant caractérisé par l'étape de fixation d'une couche de polissage non-tissée, qui comprend des fibres ayant une épaisseur de fibre jusqu'à 11 dtex et une longueur de fibre de 40 mm à 200 mm, à une couche d'attache non-tissée qui comprend des fibres ayant une épaisseur de fibre supérieure à 11 dtex et une longueur de fibre de 40 mm, par enchevêtrement de fibres des couches de polissage et d'attache.

10. Procédé suivant la revendication 9, caractérisé en ce que l'enchevêtrement est effectué par aiguilletage.

11. Procédé suivant la revendication 9 ou la revendication 10, caractérisé en ce qu'un liant est appliqué aux fibres de la couche de polissage et de la couche d'attache.
